

# UNITED STATES PATENT OFFICE.

ERNEST EMIL SCHMIDT, OF COVINGTON, KENTUCKY.

## SAFETY-PAPER.

1,217,076.

Specification of Letters Patent. Patented Feb. 20, 1917.

No Drawing.

Application filed January 26, 1916. Serial No. 74,500.

To all whom it may concern:

Be it known that I, ERNEST EMIL SCHMIDT, a citizen of the United States, residing at Covington, in the county of Kenton and State of Kentucky, have invented new and useful Improvements in Safety-Paper, of which the following is a specification.

This invention relates to paper used for checks, notes, wills, deeds, etc., and has for its object to prevent successful fraudulent alteration of matter written on such paper with commercial fluid writing ink.

For this purpose I impregnate the paper, or the pulp from which it is made, with an agent adapted to chemically combine with the essential ingredients of commercial writing ink in rendering matter written with said ink indelible either by the acid and 20 alkaline solutions usually employed to remove commercial ink from paper, or by the abrasive action of a mechanical eraser.

I have used with satisfactory results an agent composed of a solution of ferro-cyanid 25 of potassium, or its chemical equivalent, viz., ferro-cyanid of sodium, ox gall, magnesium sulfate, and water, using by preference the following proportions:

Ferro-cyanid of potassium (or ferro- 30 cyanid of sodium), two pounds,

Ox gall, three ounces,

Magnesium sulfate, one ounce,

Water, four gallons.

Any ordinary writing paper impregnated 35 with said solution becomes very sensitive to commercial writing inks, all of which contain tannate of iron or other similar preparation of iron, in quantity sufficient to make the written matter legible, and also contain 40 nut gall and tannin. The ink at once combines with the said agent and is rendered practically indelible, so that it cannot be successfully removed without detection, either by means of chemical ink eradicators 45 or by mechanical abrasion.

In eradicating commercial writing ink, two liquid solutions are applied successively or alternately to the paper, one being acid and the other alkaline. Either of said solutions alone is not capable of removing the ink without leaving evidence of fraud, but the two solutions used successively are capable of entirely removing any commercial ink from ordinary paper.

When paper treated in accordance with 55 my invention has been written upon with any ink and an attempt is made to remove the writing by an acid and an alkali, the following chemical changes take place:

If an acid is used in the first step of eradicating the ink, the acid immediately sets the ink by combining with the iron and tannin of the ink and with the ferro-cyanid of potassium (or sodium) in the paper, forming ferro-cyanid of iron, which is insoluble 65 in all acids and alkalis, and is therefore indelible, and cannot be removed without destruction of the paper.

If an alkali is first used, it will similarly set the ink and render it indelible. 70

In either case the chemical action is such that evidence of fraud is plainly visible on the paper.

The ox gall incorporated in the paper has the effect of causing fluid ink to penetrate 75 or sink into the paper to such an extent as to materially increase the difficulty of successfully removing the ink from the paper by a mechanical eraser or other abrading instrumentality.

The magnesium sulfate hardens the paper and prevents the ink from creeping laterally at the surface of the paper, and thus blurring the written lines.

To further guard against fraud, I provide 85 the paper with coloring matter, preferably by adding anilin dye to the solution above described, in sufficient quantity to impart the desired tint or color. The anilin dye combines with any ink-eradicating chemical 90 that may be applied to the paper, the result being a strongly contrasting color wherever the eradicator touches the paper, entirely defeating the fraudulent intent.

The dye may be applied only to the external surface of the paper, so that the color of the surface contrasts with that of the body of the paper. Mechanical erasure therefore removes the surface color and exposes a patch of contrasting color. If now 100 an attempt is made to again color the exposed patch, any coloring matter used will so combine with the chemical agent in the paper as to produce a different color from that intended and thus defeat the fraudulent intent.

I do not limit myself to the use of an anilin dye or color, and may use any pigment

suitable for the purpose. If white paper is preferred, the coloring matter may be omitted.

Having described my invention, I claim:

- 5 1. Paper impregnated with ox-gall.
2. Paper impregnated with ox-gall, and an agent adapted to combine with commercial writing ink in rendering matter written with such ink indelible.
- 10 3. Paper impregnated with ferro-cyanid and ox-gall.
4. Paper impregnated with ox-gall and magnesium sulfate.
- 15 5. Safety paper impregnated with a solution of ferro-cyanid of potassium or its

specified equivalent, ox gall, and magnesium sulfate.

6. Safety paper impregnated with a solution of ferro-cyanid of potassium or its 20 specified equivalent, ox gall, and magnesium sulfate, the paper being treated with coloring matter which is changeable by acid and alkaline ink eradicators.

7. Safety paper impregnated with a solution of ferro-cyanid of potassium or its 25 specified equivalent, ox gall, magnesium sulfate, and anilin coloring matter.

In testimony whereof I have affixed my signature.

ERNEST EMIL SCHMIDT.